

# United States Patent Office

3,223,637

Patented Dec. 14, 1965

1

3,223,637

ESTERS AND COMPOSITIONS CONTAINING SAME  
 John J. Barch, Crestwood, N.Y., and William M. Kraft,  
 Verona, N.J., assignors to Tenneco Chemicals, Inc.  
 No Drawing. Filed July 24, 1964, Ser. No. 385,045  
 6 Claims. (Cl. 252—56)

This invention relates to a novel combination of esters and to lubricant compositions containing such esters.

With the development of jet aircraft engines that operate at extremely high altitudes and at high speeds there has been a need for lubricants having a combination of properties not possessed by conventional lubricants including mineral lubricating oils. To be useful in jet aircraft engines, the lubricant must provide good lubricity and must meet a number of rigid requirements including low pour point, high flash point, and viscosity requirements. In the past, esters prepared from a variety of alcohols and acids have been suggested as lubricants; however, most of these esters do not have the properties required for jet engines. Esters of neopentyl alcohols and monobasic acids or monobasic and dibasic acids have been suggested which meet the requirements of the less stringent specifications, for example, Military Specification MIL-L-7808, but do not meet the requirements of the more stringent Military Specification MIL-L-23699.

A combination of two esters has been discovered that meets the requirements of base fluids for MIL-L-23699 lubricants. The combinations of esters contains from 67 to 73 parts of trimethylolpropane tripelargonate and from 33 to 27 parts of pentaerythritol dipelargonate di-2-methylpentanoate in each 100 parts by weight of these two esters. This combination of esters meets the requirements including the low temperature stability requirements, although neither one of these esters alone meets the low temperature stability requirements.

The esters may be readily produced in a conventional manner. The trimethylolpropane ester can be produced by reacting three moles of pelargonic acid with one mole of the alcohol,  $C_2H_5C(CH_2OH)_3$ . The pentaerythritol ester can be produced by reacting one mole of this alcohol, either sequentially or simultaneously, with two moles of pelargonic acid and two moles of 2-methylpentanoic acid. Equivalent amounts of alcohol and acid or an excess of either may be used in the reaction. The reaction may be effected in the absence or presence of an esterification catalyst, for example, p-toluenesulfonic acid. The product of the esterification may be purified by conventional procedures. For example, unreacted acid may be removed by washing with a dilute alkaline solution, volatile impurities by distillation, and certain other impurities by treatment with activated carbon.

The combination of trimethylolpropane and pentaerythritol esters may be used directly as lubricants or the esters may be blended with other base fluids to obtain lubricants containing a major amount of the esters and having special characteristics. It also may be desirable to add to the esters minor amounts of certain of the well known lubricant additives such as viscosity index improvers, pour point depressors, detergents, and corrosion inhibitors. In general it is desirable to add antioxidants, for example, phenyl- $\alpha$ -naphthylamine, 2,2'-dipyridylamine, phenothiazine, or mixtures thereof. A preferred antioxidant is a mixture of phenyl- $\alpha$ -naphthylamine and a metal chelate which may be prepared from salicylaldehyde or 5-nitro-salicylaldehyde, an amine, and the metal as the chloride in the manner described in Shriner and Fuson, "Systematic Identification of Organic Compounds," 4th edition, page 125. Representative, but not the only amines, are aniline, p-phenoxyaniline, p-phenoxyphenoxy aniline, o-toluidine, o-chloroaniline, and 2-ethylhexylamine. The metal may be nickel, cobalt, or zinc. Mix-

2

tures of the chelates may be used or mixtures of the chelates and other antioxidants may be used. A preferred antioxidant is a mixture of phenyl- $\alpha$ -naphthylamine and a nickel chelate. The aforementioned chelates may be represented by the formula:



wherein Y represents  $NO_2$  or H; M represents Ni, Co, or Zn; R represents



or



and X represents H,  $CH_3$ , or Cl.

In the following examples all percentages and parts are by weight. The tests on the various compositions were made in accordance with the Military Specification MIL-L-23699 (WEP), June 6, 1963, Lubricating Oil, Aircraft Turboprop and Turboshaft Engines, Synthetic Base. All viscosities are expressed in centistokes.

## EXAMPLE 1

A lubricant composition was prepared by mixing the following materials:

70 parts trimethylolpropane tripelargonate  
 30 parts pentaerythritol dipelargonate di-2-methylpentanoate  
 2 parts phenyl- $\alpha$ -naphthylamine  
 0.2 part nickel bis(N-phenyl-5-nitrosalicylimine)

A portion was cooled to  $-40^{\circ}$  F. and the viscosity determined, ASTM D445, with the following results:

|               | Cs.   |
|---------------|-------|
| Initial       | 7,298 |
| After 3 hours | 7,298 |
| After 7 hours | 8,042 |

There was no crystallization upon standing at this low temperature.

## EXAMPLE 2

Trimethylolpropane tripelargonate alone and combinations of this ester and antioxidants were tested for crystallization upon standing at  $-40^{\circ}$  F. The amounts of antioxidant and ester set forth in the following table are parts by weight:

Table I

|                                          | Compositions |        |     |        |
|------------------------------------------|--------------|--------|-----|--------|
|                                          | A            | B      | C   | D      |
| Trimethylolpropane tripelargonate        | 100          | 100    | 100 | 100    |
| Phenyl- $\alpha$ -naphthylamine          | 2            | 3      | 3   | 0.12   |
| Nickel bis(N-phenyl-5-nitrosalicylimine) |              |        |     | 0.12   |
| Total                                    | 100          | 102.12 | 103 | 103.12 |

Crystals appeared in each of the compositions after being held for about three hours at  $-40^{\circ}$  F.

## EXAMPLE 3

Base fluids of pentaerythritol dipelargonate di-2-methyl pentanoate alone and this ester with antioxidant were cooled to  $-40^{\circ}$  F. and were found to crystallize and not meet the specification for stability at this temperature. The base fluid containing antioxidant contained 2% phenyl- $\alpha$ -naphthylamine, 0.3% nickel bis(N-phenyl-5-nitrosalicylimine), and 0.3% nickel bis(N-phenyl salicylimine).

## EXAMPLE 4

Base fluids were prepared containing both trimethylol-propane tripelargonate and pentaerythritol dipelargonate di-2-methylpentanoate in addition to antioxidants. These fluids were tested for stability against crystallization at  $-40^{\circ}$  F. None of the fluids were stable for 72 hours as required.

The compositions, parts by weight, were as follows:

Table II

|                                                     | Compositions |       |       |       |
|-----------------------------------------------------|--------------|-------|-------|-------|
|                                                     | E            | F     | G     | H     |
| Trimethylolpropane tripelargonate                   | 75           | 65    | 60    | 55    |
| Pentaerythritol dipelargonate di-2-methylpentanoate | 25           | 35    | 40    | 45    |
| Phenyl- $\alpha$ -naphthylamine                     | 0.2          | 0.2   | 0.2   | 0.2   |
| Nickel bis(N-phenyl-5-nitrosalicylimine)            |              |       |       |       |
| Total                                               | 102.2        | 102.2 | 102.2 | 102.2 |

None of the above fluids were stable for 72 hours at  $-40^{\circ}$  F. Crystals formed in Composition H after three hours and Composition G after 24 hours. Compositions E and F did not develop crystals until after 40 hours and 5 48 hours, respectively.

## EXAMPLE 5

A lubricant composition was prepared by mixing the following ingredients.

| 10 | Base fluid:                              | Parts |
|----|------------------------------------------|-------|
|    | Mixed esters                             | 99    |
|    | Polyester                                | 1     |
| 15 | Total                                    | 100   |
| 20 | Antioxidant:                             |       |
|    | Phenyl- $\alpha$ -naphthylamine          | 2     |
|    | Nickel bis(N-phenyl-5-nitrosalicylimine) | 0.2   |
| 25 | Total                                    | 2.2   |

NOTE.—The mixed esters consisted of 70% trimethylol tripelargonate and 30% pentaerythritol dipelargonate di-2-methylpentanoate. The polyester was prepared by reacting under esterification conditions one mole of pentaerythritol, 0.75 mole of succinic anhydride, and 2.5 moles of pelargonic acid.

The foregoing lubricant was subjected to various tests with the results being set forth in the following table:

30

Table III

| Test                                                                              | Results               | Specification Requirements MIL-L-23699 (Wep) |
|-----------------------------------------------------------------------------------|-----------------------|----------------------------------------------|
| Viscosity, cs. (ASTM D445):                                                       |                       |                                              |
| At $210^{\circ}$ F.                                                               | 5.02                  | 5.0 min.—5.5 max.                            |
| At $100^{\circ}$ F.                                                               | 25.82                 | 25 min.                                      |
| At $-40^{\circ}$ F.                                                               | 7,545                 | 13,000 max.                                  |
| Stability at $-40^{\circ}$ F.:                                                    |                       |                                              |
| After 3 hours, percent viscosity change                                           | 0                     | 6 max.                                       |
| After 72 hours, cs.                                                               | 8,032                 | 17,000 max.                                  |
| Flash point (ASTM D92)                                                            | 475° F.               | 425° F. min.                                 |
| Pour Point (ASTM D97)                                                             | -75° F.               | -65° F. max.                                 |
| Total Acid No.                                                                    | 0.24                  | 0.5 max.                                     |
| Evaporation Loss (ASTM D972), 6.5 Hours, $400^{\circ}$ F., atmospheric pressure.  | 3.1%                  | 20% max.                                     |
| Lead Corrosion (SOD), mg./sq. in. loss, 1 hour at $325^{\circ}$ F.                | 4.8 mg.               | 6 mg. max.                                   |
| Foaming, M1. foam after 5-minute blow period—settling period to zero volume foam: |                       |                                              |
| Seq. I ( $75^{\circ}$ F.)                                                         | 20 ml.—10 sec.        | 25 ml.—60 sec. max.                          |
| Seq. II ( $200^{\circ}$ F.)                                                       | 10 ml.—15 sec.        | 25 ml.—60 sec. max.                          |
| Seq. III ( $75^{\circ}$ F.)                                                       | 20 ml.—10 sec.        | 25 ml.—60 sec. max.                          |
| Rubber (H) swell, percent change                                                  | 11.43                 | 15% min.—35% max.                            |
| Thermal Stability:                                                                |                       |                                              |
| Viscosity change, percent of original at $100^{\circ}$ F.                         | +0.8%                 | $\pm 5\%$ .                                  |
| Total Acid No. change                                                             | 1.9                   | 2 max.                                       |
| Appearance                                                                        | Dark, no precipitate. | No insolubles, phase separation or sediment. |
| Storage Stability at $230^{\circ}$ F.:                                            |                       |                                              |
| 48 Hour lead loss, mg./sq. in.                                                    | 5.87                  | 25 max.                                      |
| 168 Hour lead loss, mg./sq. in.                                                   | 6.50                  | 150 max.                                     |
| Shear Stability, percent Viscosity loss at $100^{\circ}$ F.                       | 0.4                   | 4 max.                                       |
| Corrosion and Oxidation Stability:                                                |                       |                                              |
| After 72 Hours at $100^{\circ}$ F.:                                               |                       |                                              |
| Percent Viscosity change at $100^{\circ}$ F.                                      | +11.8%                | -5 to +15%.                                  |
| Total Acid No. change                                                             | 0.07                  | 2.                                           |
| Metal Wt. Change, mg./sq. in.:                                                    |                       |                                              |
| Steel                                                                             | 0.0                   | $\pm 0.2$ .                                  |
| Silver                                                                            | 0.0                   | $\pm 0.2$ .                                  |
| Aluminum                                                                          | 0.0                   | $\pm 0.2$ .                                  |
| Magnesium                                                                         | 0.0                   | $\pm 0.2$ .                                  |
| Copper                                                                            | 0.07                  | $\pm 0.4$ .                                  |
| After 72 Hours at $400^{\circ}$ F.:                                               |                       |                                              |
| Percent Viscosity change at $100^{\circ}$ F.                                      | +25%                  | -5 to +25%.                                  |
| Total Acid No. change                                                             | 2.1                   | 3.                                           |
| Metal Wt. Change, mg./sq. in.:                                                    |                       |                                              |
| Steel                                                                             | 0.0                   | $\pm 0.2$ .                                  |
| Silver                                                                            | 0.0                   | $\pm 0.2$ .                                  |
| Aluminum                                                                          | 0.0                   | $\pm 0.2$ .                                  |
| Magnesium                                                                         | 0.0                   | $\pm 0.2$ .                                  |
| Copper                                                                            | 0.09                  | $\pm 0.8$ .                                  |
| Ryder Gear Test Average 4 Determinations, percent Reference Oil B.                | 98.2                  | 88 min.                                      |

The lubricating oil met all of the above-mentioned major requirements and met all of the minor requirements except for the minimum rubber swelling requirement which is a relatively minor requirement and not one to rule out use of the lubricant.

The small amount of polyester was included to effect a slight increase in the viscosity at 210° F. as the base fluid without the polyester was borderline as to meeting this test. Small amounts of other relatively more viscous esters, usually constituting less than 10% of mixed esters of the present invention, may be used for the same purpose.

What is claimed is:

1. A composition comprising from 67 to 73 parts of trimethylolpropane tripelargonate and from 33 to 27 parts of pentaerythritol dipelargonate di-2-methylpentanoate per 15 each 100 parts total weight of trimethylolpropane tripelargonate and pentaerythritol dipelargonate di-2-methylpentanoate.

2. A composition comprising 70 parts by weight of trimethylolpropane tripelargonate and 30 parts by weight of 20 pentaerythritol dipelargonate di-2-methylpentanoate.

3. A lubricant composition comprising a base fluid, at least 50% of the base fluid consisting of the combination of from 67 to 73 parts by weight of trimethylolpropane tripelargonate and from 33 to 27 parts by weight of pentaerythritol dipelargonate di-2-methylpentanoate.

4. A lubricant composition comprising base fluid and antioxidant for the base fluid, at least 90% of the base fluid consisting of the combination of from 67 to 73 parts by weight of trimethylolpropane tripelargonate and from 33 to 27 parts by weight of pentaerythritol dipelargonate di-2-methylpentanoate.

5. A lubricant composition comprising base fluid essentially composed of 70 parts by weight of trimethylolpropane tripelargonate and 30 parts by weight of pentaerythritol dipelargonate di-2-methylpentanoate.

6. A lubricant composition comprising antioxidant and base fluid containing in each 100 parts about 99 parts of a mixture of esters and about 1 part of polyester resulting from the esterification of 1 mole of pentaerythritol with about 0.75 mole of succinic anhydride and about 2.5 moles of pelargonic acid, said mixed esters essentially consisting of 70% by weight of trimethylol tripelargonate and 30% by weight of pentaerythritol dipelargonate di-2-methylpentanoate.

#### References Cited by the Examiner

##### UNITED STATES PATENTS

|           |         |                 |       |          |
|-----------|---------|-----------------|-------|----------|
| 2,615,860 | 10/1952 | Burgess         | ----- | 260—429  |
| 2,991,297 | 7/1961  | Cooley et al.   | ----- | 252—56 X |
| 3,000,827 | 9/1961  | Moler           | ----- | 252—56   |
| 3,000,917 | 9/1961  | Babayan.        |       |          |
| 3,036,005 | 5/1962  | Koch            | ----- | 252—49,6 |
| 3,065,180 | 11/1962 | Pethrick et al. | ----- | 252—56   |

##### OTHER REFERENCES

Calvin et al.: The Oxygen-Carrying Synthetic Chelate Compounds, *Journal of the American Chemical Society*, vol. 68 (1946), pp. 2267—2273.

Marvel et al.: Heat Stability Studies on Chelates From Schiff Bases of Salicylaldehyde Derivates, *Journal of the American Chemical*, vol. 80 (1958), pp. 832—835.

DANIEL E. WYMAN, *Primary Examiner.*